

Patented Mar. 1, 1927.

## UNITED STATES PATENT OFFICE.

HERBERT L. JOHNSON, OF BROOKLYN, NEW YORK, ASSIGNEE TO STANDARD DEVELOPMENT COMPANY, A CORPORATION OF DELAWARE.

## LUBRICANT.

No Drawing.

Application filed November 24, 1923. Serial No. 676,853.

This invention relates to lubricants and their preparation and more particularly lubricants which can be used where water is present.

5 In the refining of mineral oils by treating with fuming or concentrated sulfuric acid there are formed certain hydrocarbon sulfonic acids. Some of these are oil-soluble, and water-insoluble, and others 10 are water-soluble but insoluble in oil. These latter separate and settle out of the oil as sludge, while the oil-soluble acids have to be removed from the oil by special treatments. It has been proposed 15 to use lubricating oil containing the oil-soluble sulfonic acid already present, as a lubricant for some uses; but the water-soluble or sludge sulfonic compounds although showing indications of superior lubricating 20 qualities of promise for certain uses have remained a waste sludge material because not capable of being dissolved in oil.

I have now found that by a suitable procedure I can incorporate the water-soluble sulfonic compounds in oil and thus attain a wide range of lubricants available for uses not heretofore reached by mineral oils.

While for some uses I may employ the water-soluble free sulfonic acid for making up lubricants in accordance with the present invention, I ordinarily prefer the salts thereof or sulfonates, and taking for example a sulfonic acid separated in the sludge after treating a petroleum lubricating oil 30 with a 5-10% dump of fuming sulfuric acid, and such sulfonic acid being then purified by salting out of a water solution and neutralized with caustic soda, I first dry or dehydrate such sodium sulfonate product. After 35 dehydrating I dissolve or incorporate the water-soluble sodium sulfonate in a non-mineral oleaginous vehicle, such for example as corn oil, sulfurized corn oil, lard oil, soya bean oil or oleic acid. Such vehicle takes up the sulfonate in high degree, for instance I can incorporate 5-20 parts by weight of the dehydrated water-soluble sodium sulfonate with 5 parts by weight of oleic acid. Ordinarily I prefer 10-15 parts of the sulfonate to 5 parts of the oleic acid with mineral oils of 200-300 seconds Saybolt viscosity at 40 100° F.; and with mineral oils of 100-150 seconds Saybolt viscosity at 100° F., 5% of the sulfonate and 10% of oleic acid may be used. 45 The water-soluble sodium sulfonate in its oleaginous vehicle is now incorporated in mineral oil, for example a green cylinder stock or any desired petroleum lubricating oil preferably over 90 seconds Saybolt viscosity at 100° F. The proportions of mineral oil and oleaginous vehicle containing the sulfonic compound may vary within considerable limits depending upon the particular use in view, but an illustrative formula is 10% of water-soluble sodium sulfonate, 5% of oleic acid, and 85% of mineral lubricating oil. For example, water-soluble sodium sulfonate is dried in a steam jacketed kettle or pan until the water content is reduced to at least about 2%, and the material 50 becomes brittle in texture. Sufficient of the dried sulfonate to make 10% by weight in the finished product is then put in a steam jacketed mixing kettle and oleic acid sufficient to make 5% in the finished product is 55 added, together with mineral oil amounting to about 10% on the finished product. This addition of mineral oil is for thinning the mass to facilitate working and it may be a relatively thin oil, for instance 65 seconds 60 Saybolt viscosity at 100° F. On stirring and heating to about 250° F., the sulfonate melts and dissolves. Mineral oil is now added 65 gradually to bring the composition up to 100%, the mineral oil having a viscosity 70 such that the resulting product will have a consistency best suited for its specific use. If the sulfonate used contained any dirt or salt, the fluid mixture is now filter-pressed 75 or otherwise separated from sediment. One 80 finished formula which is advantageous contains for instance 10% by weight of the anhydrous sodium sulfonate, 5% of oleic acid, 85 60% of a petroleum oil of about 65 seconds Saybolt viscosity at 100° F., and 25% of a 90 petroleum oil cylinder stock to bring up the 95 viscosity.

Where desired, for certain uses, rosin oil, usually about 3-5%, can be added. For instance, oleic acid, 2.5% based on the finished product, and all of the anhydrous sodium sulfonate (e. g. 5% for the latter based on the finished product) and a small amount of petroleum lubricating oil (e. g. 5%) are heated and mixed in a kettle until the sulfonate is dissolved. While cooling, about 5% of rosin oil and the rest of the oleic acid (i. e. about 5%) and the rest of the petroleum lubricating oil (i. e. about 74%) are mixed in another kettle and 110

heated slightly and about 1.24% of saturated potassium hydroxid solution is added to neutralize a part of the acid constituents in the ultimate product. The sulfonate mixture from the first kettle is then added to the second mixture and the whole well mixed. About 2-2.5% of an alcohol (e. g. ethyl or isopropyl alcohol) is then added and stirred. The product is filtered if necessary. As an alternative to the above example, the total quantity of oleic acid may be mixed with the sulfonate and oleic acid will then be omitted from the mixture in the second kettle. In some cases other alkalies can be substituted for the potassium hydroxid. Oils have been compounded with the following variations in composition:

79-84% petroleum lubricating oil, 3-5% water soluble sodium sulfonate, 5-7.5% oleic acid, 3-5% rosin oil, the whole mixture neutralized with a basic potassium compound and 2-3% of an alcohol added.

By using more sulfonate, also additional soaps if desired of rosin or fatty acids with sodium or potassium or calcium bases, lubricants of various consistency for greases can also be prepared.

Where desired, ordinary mineral oils may be substituted in whole or in part by sulfurized oils, as for example cylinder stock petroleum oil into which sulfur has been cooked to an extent of 0.5 to 3% or more combined sulfur. Thus, one advantageous formula for a cutting oil is 10% of anhydrous sodium sulfonate, 5% of oleic acid, 60% of a petroleum oil of about 65 seconds Saybolt viscosity at 100° F., and 25% of a highly sulfurized cylinder stock. The combined sulfur in the oil of this formula is not less than 0.25%.

While I have described my invention by reference to certain specific details it is to be understood that these are for the purpose of illustrating the practice of the invention and are not limitative, and I intend to claim all inherent novelty as broadly as the prior art permits.

What I claim is:

1. The process of preparing lubricants, which comprises dissolving about 5 parts by weight of a dehydrated water-soluble sodium sulfonate in about 2.5 parts of oleic acid and about 5 parts of petroleum lubricating oil, and mixing with about 5 parts of rosin oil about 5 parts of oleic acid and about 74 parts of petroleum lubricating oil and about 1.24 parts of saturated potassium hydroxid solution and finally adding about 2.5 parts of isopropyl alcohol to the whole.

2. The process of preparing lubricants, which comprises mixing a dehydrated sodium sulfonate derived from mineral oils in oleic acid and a petroleum lubricating oil and adding a small proportion of an alcohol.

3. The process of preparing lubricants, which comprises incorporating a dehydrated sulfonate derived from mineral oils in a non-mineral oil vehicle and a petroleum lubricating oil together with a small proportion of an alcohol.

4. The process of preparing lubricants, which comprises incorporating 5-20 parts by weight of a dehydrated water-soluble sodium sulfonate derived from mineral oils with about 5 parts of a non-mineral oleaginous vehicle and admixing with 3-5 parts of rosin oil and a mineral lubricating oil to make up to 100 parts.

5. The process of preparing lubricants, which comprises incorporating a water-soluble hydrocarbon sulfonic compound with a non-mineral oleaginous vehicle, and admixing with a mineral lubricating oil.

6. In the preparation of lubricants, the improvement which comprises incorporating a substantially anhydrous hydrocarbon sulfonic compound with a hydrocarbon oil, and a small proportion of an alcohol.

7. A lubricant which comprises 79-84% of petroleum lubricating oil, 3-5% of dehydrated water-soluble sodium sulfonate derived from mineral oils, 5-7.5% of oleic acid, 3-5% of rosin oil the whole neutralized by a basic potassium compound and 2-3% of an alcohol.

8. A lubricant which comprises a mineral lubricating oil of at least 90 sec. viscosity Saybolt at 100° F., containing about 10% by weight of a substantially anhydrous water-soluble sodium sulfonate derived from mineral oils, about 5% of oleic acid, and a small proportion of rosin oil.

9. A lubricant which comprises a mineral lubricating oil containing 5-20% of a substantially anhydrous water-soluble sodium sulfonate derived from mineral oils, and about 5% of a non-mineral oleaginous vehicle.

10. A lubricant which comprises a mineral lubricating oil containing a water-soluble sulfonic compound derived from mineral oils and a non-mineral oleaginous vehicle.

11. A cutting oil which comprises 10% of a hydrocarbon sulfonic material, 5% of oleic acid, 60% of petroleum lubricating oil, and 25% of a highly sulfurized cylinder stock.

HERBERT L. JOHNSON.